

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## ALLOY

No Drawing.

Application filed May 13, 1930. Serial No. 452,131.

The invention comprises a group of substantially nickel-free alloys which contain iron as the preponderating constituent, and which also contain chromium, manganese and molybdenum as essential constituents.

In my application Serial No. 435,957, filed March 14, 1930, I have shown that ferrous alloys containing sufficient chromium, say 15% to 22%, to render them strongly <sup>55</sup> resistant to corrosion, can be advantageously modified by adding manganese, so that the manganese content of the complete alloy will fall, for example, between 6% and 16%. It has heretofore become an extensive practice <sup>10</sup> to modify corrosion-resistant binary iron-chromium alloys by incorporating nickel, but the addition of nickel impairs the resistance of the alloy to the action of sulphur-bearing gases. Manganese gives the high degree of <sup>15</sup> workability and the other properties imparted by nickel, but without evoking susceptibility to attack by sulphur-containing gases.

I have now discovered that if both manganese and molybdenum are added to a corrosion-resistant iron-chromium base, the alloys produced have properties especially adapting them to certain uses. Articles fabricated from these new alloys resist corrosion <sup>20</sup> at elevated temperatures at least as well as the ternary iron-chromium-manganese alloys; while the strength at elevated temperatures is materially enhanced by the presence of the molybdenum.

The invention is not restricted to the incorporation of any particular proportion of molybdenum. Doubtless very small additions of molybdenum produce an effect, but it is my present opinion that at least 1% will be required, as a rule, to impart the desired <sup>25</sup> qualities. Also, the quantity added will usually not exceed 10%, but useful alloys can certainly be made with higher percentages of molybdenum.

In the softest and most ductile grades of <sup>30</sup> the alloys under discussion, carbon is not an essential constituent, and it is present only because it is commercially impossible completely to exclude it. Alloys with less than 0.12% carbon are especially suitable for some uses. Greater strength and hardness can be

imparted by the incorporation of more carbon, and without much impairment of the stain-resistance and workability, but for the applications of the alloy herein contemplated, the carbon is preferably held below <sup>55</sup> a maximum of about 0.3%.

The effect of molybdenum is particularly advantageous when the alloy is used at temperatures materially below 900° C. There are many fields of use in which the temperatures encountered are in the vicinity of 600° C., and at such temperatures the molybdenum-containing alloys are decidedly stronger than similar alloys free from this metal. The merit of the new alloys in this respect is best <sup>60</sup> illustrated by measurements of yield point made at 600° C., and typical numbers are shown in the following table:

| Composition |       |       |       |      | Yield point at<br>600° C.   | 70 |
|-------------|-------|-------|-------|------|-----------------------------|----|
| Cr          | Ni    | Mn    | Mo    | C    |                             | 75 |
| 17.71       | 8.50  | 0.48  | ----- | 0.15 | 14,000 lb./in. <sup>2</sup> |    |
| 17.17       | ----- | 8.09  | ----- | 0.06 | 18,000 lb./in. <sup>2</sup> |    |
| 17.19       | ----- | 10.27 | ----- | 0.11 | 20,000 lb./in. <sup>2</sup> |    |
| 17.68       | ----- | 8.79  | 3.07  | 0.09 | 31,000 lb./in. <sup>2</sup> |    |
| 17.62       | ----- | 8.59  | 5.26  | 0.08 | 33,500 lb./in. <sup>2</sup> |    |

Among the more important fields of use for the new alloys may be mentioned the fabrication of tubes for the pyrolysis or cracking of hydrocarbon material, e. g. the cracking of petroleum fractions for the manufacture of gasoline; and the construction of supporting structures for such tubes. <sup>80</sup> <sup>85</sup>

I claim:

1. A ferrous alloy characterized by high resistance to sulphur-containing gases and by high strength at elevated temperatures in the vicinity of 600° C., and which has <sup>90</sup> substantially the composition: chromium from about 16% to about 22%, manganese from about 6% to about 16%, molybdenum from about 1% to about 10%, and carbon, the carbon content being less than about 0.3%, the balance being iron. <sup>95</sup>

2. A ferrous alloy characterized by high resistance to sulphur-containing gases and by high strength at elevated temperatures in the vicinity of 600° C., and which has <sup>100</sup>

substantially the composition: about 18% of chromium, about 8% of manganese, from about 1% to about 10% of molybdenum, and carbon, the carbon content being less than about 0.3%, the balance being iron.

3. A ferrous alloy characterized by high resistance to sulphur-containing gases and by high strength at elevated temperatures in the vicinity of 600° C., and which has substantially the composition: chromium from about 16% to about 22%, manganese from about 6% to about 16%, molybdenum from about 3% to about 10%, and carbon, the carbon content being less than about 0.3%, the remainder iron.

4. A ferrous alloy characterized by high resistance to sulphur-containing gases and by high strength at elevated temperatures in the vicinity of 600° C., and which has sub-

20

stantially the composition: chromium from about 16% to about 22%, manganese from about 6% to about 16%, molybdenum from about 1% to about 10%, and carbon, the carbon content being less than about 0.12%, the balance being iron.

5. A ferrous alloy characterized by high resistance to sulphur-containing gases and by high strength at elevated temperatures in the vicinity of 600° C., and which has sub-

75

stantially the composition: chromium from about 16% to about 22%, manganese from about 6% to about 16%, molybdenum from about 3% to about 10%, and carbon, the carbon content being less than about 0.12%, the remainder iron.

In testimony whereof, I affix my signature.

FREDERICK M. BECKET.

85

25

90

30

95

35

100

40

105

45

110

50

115

55

120

60

125

65

130